

# UNITED STATES PATENT OFFICE.

ROBERT W. EARLE, OF CHICAGO, ILLINOIS, ASSIGNOR TO THE DOVER MANUFACTURING COMPANY, OF DOVER, OHIO, A CORPORATION OF OHIO.

## ELECTRICAL INSULATING AND HEAT-CONDUCTING MATERIAL.

1,402,750.

Specification of Letters Patent. Patented Jan. 10, 1922.

No Drawing.

Application filed June 27, 1918. Serial No. 242,250.

To all whom it may concern:

Be it known that I, ROBERT W. EARLE, a citizen of the United States, resident of Chicago, county of Cook, and State of Illinois, 5 have invented new and useful Improvements in Electrical Insulating and Heat-Conducting Material, of which the following is a specification, the principle of the invention being herein explained and the best mode 10 in which I have contemplated applying that principle, so as to distinguish it from other inventions.

My invention relates to electrical insulating and heat conducting material for sad 15 irons, soldering irons, stoves and other heating devices, such as described in my pending application Serial No. 196,610, filed October 15, 1917.

The object of my invention is to provide 20 a material of the above-described character from which uniform results may be obtained and the various units thereof made to conform to a maximum commercial standard 25 of dielectric strength, heat conductivity and durability.

It has long been known that certain clays such, for example, as fire clay, possess considerable dielectric strength. Also, that alumina or aluminum oxide clays, such as bauxite, 30 may be crystallized by fusion and that the resulting mass will not only be highly dielectric, but will have a high degree of heat conductivity. Electrical heating units have been formed by crushing the fused 35 mass into granular form, grading the crushed material by means of a screen, and then combining the material which passes through the latter with a small quantity of unfused clay which serves as a binder, after 40 which the mixture may be rendered plastic by the addition of water, resistance wires embedded therein and the unit thus formed molded to the required shape, compressed in a container to secure intimate contact with 45 the wire and the walls of the container, and baked in the form of a brick, from which the ends of the wire protrude in a position to serve as terminals.

Some of the units formed in this manner 50 have been sufficiently successful for commercial purposes. They usually possess substantially the same coefficient of expansion and contraction as that of the metal containers in which they are placed. Some of

the units have been found to possess high 55 dielectric strength. In some of them, the dielectric strength has been found to be so low that danger existed of serious shock to the persons handling the metal containers, due to current leakage from the resistance 60 wire through the embedding material to such containers. It has also been found that while some of the units retained the brick form in which they were baked, under conditions of varying temperature and moisture, yet in other units, apparently made from material of the same character and quality, the embedding material would disintegrate and crumble under the conditions 65 of service and eventually permit short circuiting by allowing contact between the resistance wire and the container, or between successive convolutions of wire, or in other cases permitting deterioration of the resistance wire by exposing it to atmospheric conditions. Variations have also been noted in 70 the thermal conductivity of different units.

For the above reasons the successful exploitation and commercial use of heating 80 units of this type have been greatly jeopardized and so far as I am aware, no one has heretofore sufficiently understood either the process or the reasons why good results were obtained in some cases, followed by 85 failures in other cases.

My invention is based upon the discovery 90 that the above-mentioned variations in results are due to the fact that the materials used are not properly prepared for such use and that the process followed in the manufacture of the units, as heretofore carried on, has been such that successful results have been accidental. I have discovered that it is sometimes necessary to first prepare the material by removing therefrom foreign 95 substances, and where the latter consist of iron and other substances which may serve as conductors for the electric current such removal is in all cases desirable; that it is also necessary to use distilled water or water 100 from which current conducting salts or minerals are absent, in order to secure the best results, and also to uniformly secure high dielectric strength. I have further discovered that success is dependent upon using, within reasonable limits, definite proportions of the fused granular material and of the binding material and to subject these 105

materials to sufficient pressure, after the resistance wire has been embedded therein, to secure intimate contact between the material and the wire and with the walls of the 5 container. I have also found it necessary to predetermine the dielectric strength of the bonding material, and to subject the material of the unit to a predetermined pressure beyond which the dielectric strength 10 will not decrease. Those portions of the bonding material which dissolve and produce plasticity are thus forced into the interstices between the harder grains and the lines of conduction which would otherwise 15 extend from the resistance wire to the container through this bonding material, are thereby in a large measure either broken or greatly extended and reduced in cross-section. In this manner the electrical resisting 20 qualities of the grains of previously fused material are utilized to the best possible advantage.

I have further discovered that in order 25 to secure the best results both as to dielectric strength and heat conductivity, it is necessary to exclude moisture from the interior of the unit as far as possible, there being a tendency for such units to absorb considerable moisture from the atmosphere. 30 I have discovered that different clays used as bonding materials differ in moisture excluding qualities or effects and this is due to that portion of the clay which is capable of being dissolved or partially dissolved in 35 the water and held in colloidal like relation. This colloidal like clay content constitutes the real bond between the grains of fused bauxite when dried and baked.

In the practice of my process, I first fuse 40 a quantity of selected highly aluminous material such as bauxite, or a mixture of bauxite and clay. This fusion may be accomplished in an electric arc furnace at a temperature of about five thousand 45 (5000) or six thousand (6000) degrees Fahrenheit or more. The material thus fused or melted forms into a crystalline mass when cooled, which is then crushed into fragments. For my process these fragments 50 are reduced to a degree of fineness whereby they may be passed through a ninety (90) or one hundred (100) mesh screen, i. e., a screen having apertures between the strands of about fifty-nine ten thousandths (.0059) 55 of an inch in diameter. The material commercially known as "alundum grain" manufactured by the Norton Co., of Worcester, Massachusetts, is made in the above-described manner and I have found this to 60 be a convenient source of supply of this class of material. I then remove from this material any iron or other ingredients having marked electrical conductive qualities. The iron (or fragments containing iron) can 65 readily be removed by passing the granular

or powdered material in dry form through a magnetic separator. Chemical processes for the removal of the iron and other conductive materials may also be utilized for this purpose if desired. This granular material when made from bauxite is substantially a fused aluminum oxide. 70

I then mix with the non-magnetizable granular or powdered material above described, a quantity of bonding material 75 such as a clay in order that the mass may be baked into brick form under the conditions hereinafter described. I have discovered that the bonding material for this purpose should have the following properties, namely; high dielectric strength; a fusing point which will not be approximated or materially approached at any working temperature to which the heating unit will be subjected when in use; capability, when mixed with water, of being held in colloidal relation to make it plastic; and considerable heat conductivity. 80

By the use of materials having properties thus described, the same being prepared 90 and fabricated in the manner set forth, I produce a ceramic body of relatively high dielectric strength with sufficient mechanical strength and of good heat conductivity, which will not craze or crackle or suffer 95 destruction because of unequal expansion. This insulating material, which may be fabricated with a resistance wire into a heating unit, is distinguished from the insulating mediums which have been used, such as 100 glass, porcelain, and such natural mediums as mica, in that my insulating medium is compact without being vitrified; a condition 105 which has been thought to be incompatible with dielectric strength.

I have discovered certain grades of Illinois plastic clay known in the trade as "Illinois kaolin," which in fact is not kaolin, to answer the above requirements in a satisfactory manner for my purposes. This 110 clay resembles "kaolin" in chemical composition, is quite fine grained and very refractory, and exhibits a surprisingly high degree of plasticity. When burned, it is not white, but has a deep buff color, due no 115 doubt to the influence of the iron which may be present in a combined form, as a silicate or titinate or some other stable compound. Under both oxidizing and reducing conditions it vitrifies very slowly, due, no 120 doubt, to the fact that it contains but a trace of such fluxing ingredients as lime, magnesia, and alkalies. Such clay may be obtained in the vicinity of Union County, Illinois, and is being sold by the Illinois 125 Kaolin Co., Anna, Illinois. I use this clay in finely divided form, grading it by passing it through a screen similar to that above-described. If iron or other electrical conducting materials are found to be present 130

in the clay, these should be removed. This may be done by a magnetic, chemical or other process which will not destroy the plasticity of the material.

- 5 After the bonding material has been prepared as above-described, it is thoroughly mixed in dry form with the non-magnetizable grains of the fused bauxite to form a compact homogeneous mixture.
- 10 I have discovered that the proportions of bonding material to fused material are important. For the purpose of obtaining dielectric strength the best results are obtained by using about fifteen per cent (15%)
- 15 of bonding material to eighty-five per cent (85%) of fused material. The bonding material being less dielectric than the fused material and not being so highly heat-conductive, it is desirable to use as small a
- 20 quantity as is consistent with the production of a durable brick, and it is also desirable that this bonding material should be pocketed as far as possible in the interstices between the fused fragments or granules. It appears that where the fine-grained or dispersed constituents of the bonding material are present in relatively large proportions, a smaller amount of bonding material may be employed than otherwise, this
- 25 being due to the fact that the bond is provided by that portion of the material which is capable of forming a colloidal like relation when water is added to the mixture.

Having provided the mixture above-described, I add a quantity of distilled water, or water free from all foreign matter such as salts having any material degree of electrical conductivity. Sufficient water is added and thoroughly mixed with the material until the mass assumes a consistency whereby it may be readily worked. The precise quantity of water is not material, since my process can be carried out, either with just sufficient water to facilitate molding or forming the material within a receptacle, or the water may be in such quantity that the mixture may be poured by means of a ladle. It is desirable, however, that the mixture be sufficiently thick to prevent a conducting wire from settling by gravity or to prevent a crimped or convoluted wire from changing its position within the mixture after it has once been placed therein.

The mixture of water, fused granular material and bonding material is then placed in a receptacle or container and a suitable resistance wire or element, such as nichrome wire, of the proper length and cross-section embedded therein, the ends of the wire having previously been provided with conducting terminals of copper or other current-conducting and comparatively non-corrosive material, which are allowed to protrude from the surface of the mixture after the wire has been embedded.

A convenient mode of embedding the wire is to partially fill the container with the mixture and then press the wire into it after the wire has been shaped and annealed, or if desired, the mixture first poured into the receptacle may be allowed to partially dry and the upper portion may then be remoistened to facilitate inserting the wire. The receptacle is then additionally filled with the embedding mixture in order to completely cover all portions of the wire except the projecting terminals.

After the resistance wire has been embedded as above described, the mixture is allowed to partially dry and is then subjected to a pressure of preferably about two and a half ( $2\frac{1}{2}$ ) tons to the square inch. This pressure is calculated to be approximately the maximum pressure that the mass will withstand without reducing the dielectric strength and therefore if the character of the fused material is varied from time to time, it may also be necessary to vary to some extent, the degree of pressure, but it appears from numerous experiments which I have made that the dielectric strength of the unit is increased by applying this heavy pressure up to a certain point beyond which it decreases, this point with the mixture above-described being about five thousand (5000) pounds per square inch. The reason for this has not been up to the present time established with absolute certainty but it may possibly result from stratification of the material including the bonding material as a result of this pressure, thereby producing shorter continuous lines of the material of less dielectric strength and hence shorter conductors between the resistance element and the container.

After thus compressing the unit, the latter is allowed to dry at a comparatively low temperature until the greater portion of the moisture has been removed and in fact until the unit appears to be thoroughly dried from a superficial standpoint. The unit is then placed in a baking oven and subjected to a temperature of about twelve hundred degrees (1200) Fahrenheit, whereby it is baked in the form of a brick, the alundum grains being united with each other and the embedding material connected intimately and rigidly with the resistance wire and the walls of the container.

I am aware that embedding materials have been subjected to pressure in order to secure intimate contacts between the materials and the walls of the container and the wire. This is also accomplished in the compressing operation above described but I believe that it has not been heretofore known that the dielectric strength of such units could be increased by subjecting the material to a definite predetermined pressure. All clays contain granular materials

and it has been observed in some cases that the dielectric strength was increased by pressure, although the reasons why this was accomplished were not understood and 5 this result, i. e., the increase in dielectric strength, was not uniformly accomplished but was a result accidentally secured by an inadvertent application of sufficient pressure.

10 The Illinois plastic clay which I employ does not fuse to any appreciable extent at a temperature of less than three thousand degrees (3000°) Fahrenheit. The temperature of the resistance element in an electric heating unit of this type, under ordinary working conditions, ranges from three hundred (300) to one thousand two hundred degrees (1200) Fahrenheit. It is therefore obvious that the fusing point of 15 the bonding material is not sufficiently approached by an ordinary working temperature to materially reduce its dielectric strength. The same is true in even more marked degree of the fused fragments or 20 granules, which require about three thousand five hundred (3500) degrees, Fahrenheit in order to soften or melt them. Numerous tests which I have made have demonstrated that dielectric clays usually lose 25 their resistance very slowly as the temperature is increased, until a temperature is reached within a few hundred degrees of the point where vitrification or incipient fusion becomes noticeable, after which any 30 increase in temperature causes a rapid loss in dielectric strength. It is therefore exceedingly important in the selection of embedding materials or mixtures for embedding materials, that they be not only dielectric when cold, but that their dielectric 35 strength shall remain substantially constant at all temperatures up to maximum working temperature and sufficiently beyond that temperature to avoid material change 40 in conductivity through accidental overheating of the units. I have discovered that some materials which show great dielectric strength when cold rapidly lose this quality when subjected to an increase 45 in temperature of only a few hundred degrees Fahrenheit. I have discovered that this is true of different clays which I have tested and I believe that I am the first to select clays for the purpose of manufacturing electrical heating units with reference 50 to their dielectric strength while heated at temperatures to which they will be subjected in the use of such units and to provide a bonding clay of substantially 55 uniform dielectric strength under the varying conditions of temperature to which such 60 units are subjected.

The fused aluminum oxide grains or aluminum grains are important factors in providing a unit having the requisite heat con-

ductivity and also in providing a non-shrinking body of embedding material whereby the mixture will remain in contact with the heating element and the walls of the container during the drying process. 70 If the embedding material were composed entirely of unfused clay, there would be a considerable shrinking of the mass during the drying and baking processes and this would tend to destroy the intimate contacts 75 necessary for proper heat conductivity and would also tend to expose the heating element to atmospheric influence, particularly moisture, and would further tend to promote disintegration of the unit. The fused grains of 80 aluminum oxide do not swell or shrink under varying conditions of moisture and although the bonding material does expand with the addition of moisture and shrink when dry, yet the relatively small quantity 85 of this material present in the embedding mixture has no appreciable effect in causing the embedding material to shrink away from the wire and from the container during the drying and baking processes. In effect the 90 granular material constitutes a rigid frame held together, after the baking process, by the bonding material but sufficiently rigid under all conditions to prevent the mass 95 from shrinking away from the points of contact with the container and the resistance wire.

I have referred to the mixture of embedding material as a homogeneous mixture in the sense that the bonding material is 100 uniformly distributed throughout the mass of fused grains, but it will be observed that the embedding material of the completed unit is also homogeneous in another sense, namely, that of being one integral mass of 105 material without division lines produced by inserting the material into the container in the form of layers. This is true because no hydraulic action takes place in the mixture, after the addition of water, such as 110 might tend to solidify the mixture or cause it to set, even initially after the first layer has been inserted in the container and before the last or covering layer is applied to cover the resistance element. Even if the 115 first layer is permitted to dry in any degree before the second layer is applied, the moisture contained in the second layer will permeate the surface of the first layer to some extent and when the unit is subjected 120 to the heavy compression above-described, the moisture will be thoroughly distributed throughout the entire mass of embedding material and some portions thereof will be 125 squeezed out. This expulsion of the liquid makes it desirable that the unit be covered with dry powder or with a quantity of the dry mixture before inserting the unit into the press to avoid adhesion of the moisture to the plunger.

Having fully described my invention, what I claim and desire to secure by Letters Patent is:

1. An electrical insulating and heat-conducting material consisting of grains of high dielectric strength and thermal conductivity connected by a compact non-vitrified bonding material of high dielectric strength and high fusing point. 40
2. An electrical insulating and heat-conducting material consisting of grains of high dielectric strength and thermal conductivity connected by a compact non-vitrified bonding material having a high dielectric strength at the working temperatures of the electrical heaters in which the material is to be used, said bonding material also having a high fusing point. 45
3. An electrical insulating and heat-conducting material consisting of grains free from iron and of high dielectric strength and thermal conductivity connected by a compact non-vitrified bonding material of high dielectric strength and high fusing point. 50
4. An electrical insulating and heat-conducting material consisting of grains of high dielectric strength and thermal conductivity connected by a compact non-vitrified bonding material of high dielectric strength and high fusing point and free from iron. 55
5. An electrical insulating and heat-conducting material consisting of a highly compacted mass of grains of high dielectric strength and thermal conductivity connected by a compact non-vitrified bonding material of high dielectric strength and high fusing point. 60
6. An electrical insulating and heat-conducting material consisting of a highly compacted mass of grains of high dielectric strength and thermal conductivity connected by a non-vitrified bonding material of high dielectric strength and high fusing point, the degree of compactness being such as results from a pressure beyond which a decrease of dielectric strength would take place. 65
7. An electrical insulating and heat-conducting material consisting of grains of high dielectric strength and thermal conductivity connected by a compact bonding material consisting of non-vitrified Illinois kaolin. 70
8. An electrical insulating and heat-conducting material consisting of grains of fused aluminum oxide connected by a compact bonding material consisting of non-vitrified Illinois kaolin. 75
9. An electrical insulating and heat-conducting material consisting of a highly compacted mass of grains of high dielectric strength and thermal conductivity connected by a compact bonding material consisting of non-vitrified Illinois kaolin. 80
10. An electrical insulating and heat-conducting material consisting of a highly compacted mass of grains of high dielectric strength and thermal conductivity connected by a bonding material consisting of non-vitrified Illinois kaolin, the degree of compactness being such as results from a pressure beyond which a decrease of dielectric strength would take place. 85

Signed by me, this 18th day of June, 1918.

R. W. EARLE.